

## UNITED STATES PATENT OFFICE

2,058,423

TEXTILE MATERIAL AND THE MANU-  
FACTURE THEREOF

William Alexander Dickie, Donald Finlayson, and  
Percy Frederick Combe Sowter, Spondon, near  
Derby, England, assignors to Celanese Corpora-  
tion of America, a corporation of Delaware

No Drawing. Application June 24, 1932, Serial  
No. 619,122. In Great Britain August 22, 1931

4 Claims. (Cl. 28—1)

This invention relates to textile yarns and fabrics, and in particular to yarns capable of producing crêpe effects and fabrics exhibiting such crêpe effects. The invention is especially concerned with the use of yarns containing cellulose derivatives in the production of fabrics exhibiting crêpe or like figured effects.

It is well known that textile materials exhibiting crêpe effects are ordinarily produced by employing in their construction highly twisted yarns either in the weft or warp or both, which yarns produce a shrinking of the fabric on scouring, with the result that crêpe effects appear. Crêpe effects are, however, only obtained with difficulty by the employment of highly twisted crêpe threads of cellulose derivatives. It has, however, been found possible to produce satisfactory crêpe effects when using these materials by application to the crêpe threads and/or to the fabrics containing the crêpe threads of a substance adapted to swell the material of the threads and/or to apply a size to the threads, which size is adapted to be swollen in the scouring treatment so as to assist in the production of the crêpe effect. Such treatments are described in U. S. Patents Nos. 1,993,992 and 1,995,296 and British Patents Nos. 343,444; 348,589; 351,999; 352,451, and 357,084.

A further method which has been adopted for treating these materials is described in British Pat. No. 378,910, according to which chemical means are utilized to effect the shrinkage of the highly twisted crêpe threads in fabrics containing them. Further, it has been found that with yarns consisting of filaments of fine or very fine filament denier, for example 3, 1½—1 or less, especially if such yarns are twisted to a higher degree than usual, for example to 80—85 turns per inch or more, improved crêpe effects may be obtained. Again, it is also advantageous to apply the crêpe twist in two or more stages, between each or any of which size may be imparted to the yarns. Further, in such treatments employing two or more stages of twisting, the yarn may be treated with steam or other vapours between stages as described in British Patent No. 386,344. Yet other methods of producing crêpe threads from cellulose derivatives are described in British Pat. No. 386,344, for example by applying the requisite high degree of twist in at least two stages with intermediate wetting of the yarns with water or other aqueous liquid.

Apart from the methods referred to above it has also been found of advantage to employ yarns which have been uniformly or intermit-

tently stretched beyond the elastic limit or contain filaments which have been stretched to different extents as described in U. S. Pat. No. 1,976,201 and Br. Pat. No. 371,910.

It has now been found that a still further improvement in the crêpe effect obtainable when using yarns of cellulose derivatives can be achieved by the employment of yarns which have been shrunk with methylene chloride, chloroform, tetrachlorethane, dichlorethylene, ethyl acetate or like latent solvents for the cellulose derivative. Such yarns have an increased extensibility, which is of advantage when high twists are to be inserted, and in the employment of such yarns, not only is a good figure obtained on the fabrics, but they also have an elastic appearance, soft handle, and are very closely resembling that obtained in crêpe fabrics made from natural silk. These valuable results are obtained without the tensile strength or other valuable properties of the cellulose derivative yarns being in any way deleteriously affected. Moreover, in the application of the shrinking agents to the yarns the wide choice of conditions possible in the treatment avoids there being any undesired variation in the lustre of the yarns. The said agents, though not actually solvents for the commercial acetone-soluble cellulose acetate are capable of swelling the cellulose acetate to a very high degree. When mixed with comparatively small proportions of other agents, and particularly alcohols, which are not themselves solvents for the cellulose acetate, a solvent mixture is produced. (The methylene chloride and like agents are termed "latent solvents" for the cellulose derivative.)

The methylene chloride or like shrinking agent may be applied by any suitable means to the yarns prior to the application of the requisite high degree of twist. For example, the shrinking agent may be applied to the yarns in hanks, bobbins or other packages, or during a bobbin-to-bobbin or other winding operation, or continuously with the production of the yarn, e. g. the shrinking agent may be applied to cellulose acetate yarn continuously with its production by the dry or evaporative method.

This shrinking treatment may be applied to cellulose derivative yarns however produced, though the precise effect may vary somewhat with the particular type of yarn treated, and with its method of preparation, and the concentration of the agent used, with the ester or ether content of the cellulose ester or ether, and of course, with the particular cellulose ester or ether.

Thus for instance with the ordinary commercial acetone-soluble cellulose acetate the amount of shrinking achieved with methylene chloride may depend upon the method of preparation of the 5 yarn. It has been found that the shrinking is in general greater with the modern high tenacity wet-spun yarns than it is with the commercial dry-spun yarns, and, moreover, with the dry-spun yarns it is greater if the yarn has been previously 10 subjected to a stretching treatment. As is the case with the yarns described in British Patent No. 380,504, methylene chloride or like agent used alone produces in general a very high degree of shrinkage, and it is preferable to modify the 15 effect somewhat by the addition of suitable diluents to the methylene chloride or like agent, as for example, benzene, toluene, xylene or other cyclic hydrocarbons, benzine, petrol ether, kerosene or other hydrocarbons of the aliphatic or 20 petroleum series, carbon tetrachloride, trichloroethylene, perchlorethylene and other chlorinated or halogenated compounds which are inert or comparatively inert towards the cellulose derivative. It is preferable to restrain the high shrinking 25 action of the methylene chloride or like agent by the addition of such a diluent so as to reduce the concentration of the methylene chloride to about 60 or 70%. Benzene and carbon tetrachloride are very suitable diluents for use with 30 methylene chloride in such a concentration. If desired, the amount of shrinkage may be modified by exerting a suitable tension upon the yarn under treatment, such tension being either insufficient to prevent some shrinkage or being sufficient to 35 prevent shrinkage, the tension being subsequently decreased so as to enable the shrinkage to take place.

After the application of the shrinking agent, the yarn may, if desired, be rinsed in a liquid inert to the yarn, but forming a solvent for any 40 constituent of the shrinking liquid which would normally tend to plastify the yarn if allowed to concentrate thereon during drying. Thus for example, if chloroform is applied to the yarn in admixture with benzene, the concentration of 45 chloroform on the yarn due to the relatively rapid evaporation of benzene may be obviated by rinsing the yarn in benzene before drying. It may be desirable to lubricate the yarn before or during 50 the twisting operation. For this purpose, a lubricant may be added to the rinsing liquid, if used, e. g. 3% of olive oil in benzene may be employed for rinsing. Alternatively or in addition, a lubricant may be applied to the yarn, before or during 55 twisting, by running the yarn over wicks, rods, rollers or the like, moistened with the lubricant to be applied.

Yarns shrunk in the manner above described may be given a requisite high degree of twist in 60 any suitable manner, either in a single stage of twisting, or in two or more stages. Before or during twisting, or after winding the twisted yarns into fabrics, the sizing, swelling and scouring treatments described in the specifications 65 previously referred to may be employed to assist in improving the crêpe effect on the fabrics. It is preferable to employ yarns of fine filament denier, and preferably to twist the yarns to a high or very high degree.

70 It is possible to produce a differential shrinkage which is of advantage in the twisted yarns either by applying the shrinking agent intermittently along the length of the yarns, or by using yarns some of whose component filaments have been 75 shrunk and others not, or between whose com-

ponent filaments different degrees of shrinking have been effected. Likewise the yarns may consist of two or more different types of cellulose derivative yarn, for example wet and dry spun yarns or yarns of different esters or ethers or of different ester or ether content, and such different filaments may be shrunk with shrinking agents in concentration before incorporation in the yarns for twisting, or after such concentration. 5

Highly twisted crêpe threads consisting of 10 shrunk yarns as described above may be incorporated in the fabrics in any suitable manner. For example, the weft alone may be wholly or partially composed of such threads or the warp may also contain them. It is found particularly 15 convenient however, in general, to employ threads of relatively low twist in the warp and to employ in the weft both crêpe threads having a left-hand twist and crêpe threads having a right-hand twist. Such threads may be disposed in the fabrics 20 in any convenient manner, for example pairs of threads of left-hand twist may alternate with pairs of threads of right-hand twist. A further method of constructing the fabrics is to weave composite crêpe threads consisting of a yarn of 25 high twist doubled with a yarn of low twist, or consisting of two yarns of high but opposite direction of twist, the yarns being prepared and the fabrics subsequently treated in accordance with the processes of the invention. In this manner 30 crêpe fabrics may be readily produced without the necessity for the employment of a loom capable of weaving two different types of yarn such as is necessary when alternate picks of yarn of left-handed twist and yarn of right-handed twist are 35 to be woven. In this connection reference is made to Br. Patents Nos. 332,903 and 375,355.

Any other highly twisted or low twist yarns, e. g. of natural silk, reconstituted cellulose or unshrunk cellulose acetate or other cellulose derivative yarns may be employed in fabrics containing the highly twisted shrunk yarns according to the invention, and further any low twist yarns employed in the fabrics may themselves have been shrunk by a treatment with methylene chloride 45 or the like as described above. 40

By way of illustration the following example is given of the application of the invention to yarns of cellulose acetate. A cellulose acetate yarn of 100 denier and 42 filaments is treated with a shrinking mixture of 3 parts by volume of methylene chloride to 1 part of benzene, whereby the denier of the yarn is increased to 112 denier. The yarn is then twisted to 20 turns per inch, and steamed for 5 minutes, after which a further stage 50 of twisting is applied, bringing the total twist to 65 turns per inch. The crêpe yarn obtained has a high strength, and a high breaking extension. The yarn is woven, 72 picks per inch into a plain 55 warp of cellulose acetate yarns, of 75 denier having 120 ends per inch, two picks of left-hand twist alternating with two picks of right-hand twist. The resulting fabric is strong, has a good crêpe 60 figure, and a pleasant handle.

While the invention has been described above 65 more particularly with reference to yarns composed of or containing acetone-soluble cellulose acetate, it may be applied to yarns made from or containing other cellulose acetates or other esters, for example, cellulose formate, propionate, butyrate, nitroacetate and the like, or made from or containing cellulose ethers, for instance methyl, ethyl or benzyl cellulose, or made from or containing cellulose ether-esters. Furthermore, in addition to filaments of cellulose derivatives, the 70 75

yarns may contain filaments of other materials such as natural silk or reconstituted cellulose. Again, the cellulose derivative filaments which the yarns contain may be wholly or partially in 5 the form of staple lengths, alone or in admixture with staple fibres of other materials such as silk, wool, cotton or the like, or with continuous filaments of other materials such as silk, or reconstituted cellulose artificial silk filaments.

10. What we claim and desire to secure by Letters Patent is:

1. In the method of producing crêpe yarns by shrinking yarns containing cellulose acetate with a latent solvent for the cellulose acetate and applying a high degree of twist thereto, the steps of 15 applying to the yarns, during the treatment with said latent solvent, a tension of such a nature that the shrinking of the yarns is restricted and then decreasing the tension whereby restraint 20 upon the shrinkage of the yarns is removed.

2. Method of producing crêpe yarns, which comprises treating yarns containing cellulose derivatives with a latent solvent for the cellulose derivative, while first maintaining the yarns under 25 a tension of such a nature that shrinking of the yarns under the action of the latent solvent is restricted, then decreasing the tension so as to

remove restraint from the yarns and to permit shrinkage to take place, and then applying a high degree of twist to the shrunk yarns.

3. In the method of producing crêpe yarns by shrinking yarns containing cellulose derivatives with a latent solvent for the cellulose derivative and applying a high degree of twist thereto, the steps of applying to the yarns, during the treatment with said latent solvent, a tension of such a nature that the shrinking of the yarns is restricted 10 and then decreasing the tension whereby restraint upon the shrinkage of the yarns is removed.

4. Method of producing crêpe yarns, which comprises treating yarns containing cellulose acetate with a latent solvent for the cellulose acetate, while first maintaining the yarns under a tension of such a nature that shrinking of the 15 yarns under the action of the latent solvent is restricted, then decreasing the tension so as to remove restraint from the yarns and to permit shrinkage to take place, and then applying a high degree of twist to the shrunk yarns. 20

WILLIAM ALEXANDER DICKIE.

DONALD FINLAYSON.

PERCY FREDERICK COMBE SOWTER.

25